

# UNITED STATES PATENT OFFICE.

FREDERICK W. HORTON, OF HACKENSACK, NEW JERSEY.

## PROCESS FOR TREATING CELLULOID PRODUCTS.

1,350,157.

Specification of Letters Patent. Patented Aug. 17, 1920.

No Drawing.

Application filed January 13, 1920. Serial No. 351,196.

To all whom it may concern:

Be it known that I, FREDERICK W. HORTON, a citizen of the United States, and resident of Hackensack, in the county of Bergen and State of New Jersey, have invented certain new and useful Improvements in Processes for Treating Celluloid Products, of which the following is a specification.

My invention relates to improvements in processes for treating celluloid products, and photographic film for the recovery of valuable products therefrom, and is especially applicable to the treatment of old or waste photographic film for the recovery of silver and camphor therefrom.

The ordinary moving picture film has a photographic emulsion thereon which contains considerable quantities of silver and the celluloid film contains a considerable percentage of camphor and it is the main object of my invention to recover both of these in an efficient and simple manner.

Further objects, features and advantages will more clearly appear from the detail description given below.

As an example of a preferred form of my invention, I take 100 pounds of moving picture or other photographic film and put it in an iron wire basket and place this in an iron or steel tank containing about 55 gallons of 10 to 20% solution of caustic soda. I then heat the mixture either externally or internally in any suitable manner until reaction starts. The celluloid film goes into solution and silver is deposited or precipitated and camphor vapor is distilled off.

The iron or steel tank is suitably covered and provided with an outlet for the camphor vapor which outlet leads to any suitable form of condenser for condensing the camphor. For this purpose I may use a jet or surface condenser or the camphor vapor may be run into a water bath and the camphor collected from the surface thereof. Toward the

end of the operation I preferably raise the temperature to about boiling to make sure that all of the celluloid film is dissolved. The silver separates out as a heavy precipitate which readily settles, as distinguished from being in a colloidal condition which

would not settle readily. Some steam is given off with the camphor but this will also be condensed by the water jet or other form of condenser used. Some other products such as amyl acetate, camphor oil and other oils may be driven off and also condensed with the camphor but the camphor may be later refined by any suitable method so as to obtain the same in substantially pure form and the oils recovered therefrom. The silver deposited is separated from the solution in any well-known or suitable manner and is then smelted by any well-known or suitable method to obtain it in the form of dense metallic silver or bar silver. While I prefer to use caustic soda as a solvent it will be understood that any other suitable solvent may be used particularly other caustics or alkaline reagents. It will also be apparent that my invention in one aspect is applicable to the recovery of camphor from celluloid products even when there is no silver or other metal to be recovered, and also to the recovery of silver alone from other photographic sheet material. Some celluloid products contain zinc or other metallic oxides and these may be recovered in the form of a precipitate from the solution in much the same manner as the silver or otherwise. Many other changes and modifications may be made and the invention embodied in widely different forms, and I therefore, do not desire to be limited to the details described and desire to cover all forms coming within the scope of any one or more of the appended claims.

What I claim as new and desire to secure by Letters Patent, is:

1. The process of recovering silver from photographic film which consists in dissolving the film in caustic alkali causing the silver to be precipitated out therein, and separating the precipitated silver from the solution.

2. The process of recovering camphor and metal from celluloid and the like containing the same, which consists in heating the celluloid or the like in caustic alkali solution to dissolve the same causing the camphor to be distilled from the solution and the metal to

separate out therein as metal bearing precipitate, and separating the metal bearing precipitate from the solution.

3. The process of recovering silver and camphor from photographic film which consists in heating the film in an alkaline solution to cause the camphor to be distilled from the solution, and the silver to separate as

silver bearing precipitate, and separating the silver bearing precipitate from the solution. 10

Signed at New York in the county of New York and State of New York this 12th day of January A. D. 1920.

FREDERICK W. HORTON.